

1

3,183,132

## METHOD OF DELAYING THE IGNITION OF WHITE PHOSPHORUS INCENDIARY COMPO- SITIONS

Seymour M. Kaye, Dover, N.J., assignor to the United States of America as represented by the Secretary of the Army

No Drawing. Filed Apr. 23, 1963, Ser. No. 275,167  
6 Claims. (Cl. 149—29)

(Granted under Title 35, U.S. Code (1952), sec. 266)

The invention described herein may be manufactured and used by or for the Government for governmental purposes without the payment to me of any royalty thereon.

This invention relates to an incendiary device and particularly, to an aerosol spray incendiary device. More particularly the invention relates to an incendiary solution which is amenable to propulsion from an aerosol spray container.

In the conduct of limited warfare the use of incendiaries as an accepted tactical weapon by troops and guerrillas has long been established. Incendiary devices have also been employed from time immemorial by saboteurs and espionage agents for the purpose of destroying military facilities and documents, diplomatic papers, records, etc. Heretofore, the incendiary devices employed have been numerous and varied, ranging from the common match to the so-called Molotov cocktail. However, all have failed in one or more respects to measure up to a universally suitable incendiary, and their use has always been attended by significant disadvantages. For example, spontaneity of ignition is undesirable with respect to espionage activities since there is no allowance for lag time to permit escape prior to incendiary action. Concomitant with spontaneous ignition is the disadvantage of immediate illumination, particularly where incendiary activities are conducted at night or in darkened areas. Destruction of the incendiary device is another disadvantage where multiple ignitions are contemplated or where a failure of ignition occurs.

Accordingly, a principal object of the present invention is to provide an incendiary device, the use of which is unattended by the foregoing and other disadvantages.

Another object of the invention is to provide an improved incendiary device which is relatively small, easily portable, and reusable.

Still another object of the invention is to provide an incendiary solution which may be propelled simply and easily from an aerosol spray container.

Other objects and advantages of the invention will be obvious or appear hereinafter in the following detailed description.

In its broadest aspect the invention comprises a solution of white phosphorus as solute in a mixture of carbon disulfide and kerosene as solvent. This solution may be applied to combustible material, e.g., paper, cloth, plastics, wood, grass, brush, jungle foliage, etc., to effect incendiary action. In the initiation of the burning action, ignition of the phosphorus occurs spontaneously but only after a sufficient period of time has elapsed for evaporation of the carbon disulfide. This time period may be increased by increasing the content of kerosene. It is therefore obvious that lag time before ignition may be controlled within fairly accurate limits.

The inventive solution lends itself to simple packaging in an aerosol spray container to which a propellant, such as dichlorodifluoromethane sold under the trademark Freon 12, is added under pressure. The resultant article

2

is easily handled, readily portable, simple to use, and reusable.

Sprays of the invention which have been formulated and packaged in aerosol containers comprise the following percent by weight ranges of ingredients:

White phosphorus ----- 5 to 10%, preferably 7.5%.  
Carbon disulfide ----- 35 to 60%, preferably 47.5%.  
Kerosene ----- 10 to 30%, preferably 20%.  
Freon 12 ----- 25% 25%.

While the foregoing is illustrative of the invention, it is expressly understood that various changes may be made in the device and solution of this invention and that ingredients other than those specifically described herein may be employed without departing from the spirit and scope of this invention.

I claim:

1. A method of controllably delaying the ignition of combustible materials contacted with white phosphorus incendiary, said method comprising the steps of dissolving 6 $\frac{1}{2}$  to 13 $\frac{1}{2}$  % by weight of white phosphorus in 46% to 80% by weight of carbon disulfide to form a solution, adding to said solution increasing amounts of kerosene for increasing the amount of delay in spontaneous ignition, said kerosene ranging between 13 $\frac{1}{2}$  to 40% by weight of the resultant solution and applying the resultant solution to said combustible materials.

2. The method described in claim 1 wherein 10% by weight of white phosphorus is dissolved in 63 $\frac{1}{2}$  % by weight of carbon disulfide and 26 $\frac{1}{2}$  % by weight of kerosene.

3. A method of controllably delaying the ignition of combustible material contacted with white phosphorus incendiary, said method comprising the steps of dissolving 5 to 10% by weight of white phosphorus in 35 to 60% by weight of carbon disulfide to form a solution, adding to said solution increasing amounts of kerosene for increasing the amount of delay in spontaneous ignition, said kerosene ranging from 10 to 30% by weight, incorporating therewith 25% by weight of dichlorodifluoromethane and spraying the resultant mixture under pressure into said combustible material.

4. A method of delaying the ignition of combustible solid material with white phosphorus incendiary, comprising applying to said combustible material a solution of about 5 to 10 parts by weight of white phosphorus in about 35 to 60 parts by weight of carbon disulfide and about 10 to 30 parts by weight of kerosene; whereby spontaneous ignition of said white phosphorus is delayed until said carbon disulfide has evaporated from said solution.

5. The method described in claim 4 wherein said solution is applied from a pressurized container to said combustible material.

6. The method described in claim 5 wherein said solution is propelled from said container by dichlorodifluoromethane.

## References Cited by the Examiner

### UNITED STATES PATENTS

2,573,471 10/51 Malina et al. ----- 149—29 X  
2,747,672 5/56 Simm ----- 149—29 X  
3,010,815 11/61 Pierce et al. ----- 149—40 X

CARL D. QUARFORTH, Primary Examiner.

REUBEN EPSTEIN, Examiner.